

# UNITED STATES PATENT OFFICE.

JAMES ROOTS, OF BAKER STREET, MIDDLESEX, ASSIGNOR TO DOMEIER & CO., OF LONDON, ENGLAND.

## PROCESS OF PREPARING BURNING-OIL FOR LAMPS AND RESULTING PRODUCT.

SPECIFICATION forming part of Letters Patent No. 340,522, dated April 20, 1886.

Application filed October 26, 1885. Serial No. 180,969. (No specimens.)

*To all whom it may concern:*

Be it known that I, JAMES ROOTS, a subject of the Queen of Great Britain, residing at Baker Street, Middlesex, England, have invented certain new and useful Improvements 5 in the Process of Preparing Burning-Oils for Lamps and Resulting Product; and I do hereby declare that the following is a full, clear, and exact description of the invention, which 10 will enable others skilled in the art to which it appertains to make and use the same.

This invention has for its object improvements in the preparation of oils for burning in lamps.

15 I take the oils at present employed for burning in lamps from a wick and improve their illuminating quality by dissolving naphthaline in them in proportion of ten or fifteen per cent. Colza-oil may be improved in this way; so, 20 also, may sperm-oil and paraffine or earth oil.

In carrying out my invention I usually hasten the solution of the naphthaline in the oil by 25 the application of a gentle heat. The oil, if afterward cooled to about 40° Fahrenheit, will deposit any excess of naphthaline, if such should have been used in the preparation. The quantity of naphthaline which oils will 30 retain in solution at this temperature varies somewhat with the nature of the oil. The more volatile petroleums will retain more than the less volatile and more than colza-oil and sperm-oil.

35 In practice I have found that ten per cent., by weight, of naphthaline dissolved in animal, vegetable, and light mineral oils, and eight per cent. dissolved in the heavy mineral oils, produces the best results, as these oils hold well

these respective quantities in solution at ordinary temperatures.

The solution thus produced is burned directly 40 in lamps of such construction as commonly employed for burning the respective oils, and in the same manner as the oils alone are now burned.

The various burning-oils thus enriched by 45 dissolving naphthaline therein when used possess greater illuminating properties than the various oils when used alone.

I am aware that it has heretofore been proposed to mix solid and liquid hydrocarbons to 50 be burned with oxygen in lamps specially constructed to this end; also, to mix paraffine with tallow to make a burning-fluid, and also to mix camphor with hydrocarbon oils to deodorize them.

Having thus described my invention and acknowledged the state of the art so as to specifically ascertain my improvement, I claim—

1. The process of improving the illuminating quality of hydrocarbon fluids for burning 55 in the ordinary way in ordinary lamps, consisting in dissolving in such fluids naphthaline in proportion of from, say, eight to fifteen per cent., according to the volatility of the fluid, substantially as described.

2. The burning-fluid herein described, consisting of an admixture of hydrocarbon oil—such as petroleum, colza, or sperm—and from eight to fifteen per cent. of naphthaline.

JAMES ROOTS.

Witnesses:

EDWARD CARPENUEL,  
WILLIAM ROXBURY.